

F. BERGIUS & J. BIELWILLER.  
PROCESS FOR PRODUCING LIQUID OR SOLUBLE ORGANIC COMBINATIONS FROM HARD COAL  
AND THE LIKE.  
APPLICATION FILED AUG. 3, 1914.

1,251,954.

Patented Jan. 1, 1918.



Friedrich Bergius  
and John Bielwiller  
by  
Bergius, Bonn and Bielwiller  
atteis.

# UNITED STATES PATENT OFFICE.

FRIEDRICH BERGIUS AND JOHN BILLWILLER, OF HANOVER, GERMANY.

PROCESS FOR PRODUCING LIQUID OR SOLUBLE ORGANIC COMBINATIONS FROM HARL COAL AND THE LIKE.

1,251,954.

Specification of Letters Patent. Patented Jan. 1, 1918.

Application filed August 3, 1914. Serial No. 854,825.

To all whom it may concern:

Be it known that we, (1) Dr. FRIEDRICH BERGIUS and (2) JOHN BILLWILLER, citizens of (1) the German Empire and (2) Switzerland, (St. Gallen,) residing at Hanover, Germany, have invented certain new and useful Improvements in or Relating to Processes for Producing Liquid or Soluble Organic Combinations from Hard Coal and the like, 10 of which the following is a specification:

This invention relates to a process of treating carbonaceous material such as natural coals or other products of carbonization of wood and other vegetable matter, 15 so as to transform such carbonaceous material into a liquid or into substances of low melting point practically without leaving a solid carbonaceous residue in the form of coke or similar material. The process of this 20 invention whereby the liquefaction of coal is obtained consists therein that the coal is subjected to the action of hydrogen at high pressure of more than 20 atmospheres and elevated temperature not exceeding 600° 25 centigrade, preferably at a hydrogen pressure of more than 40 atmospheres, and at an elevated temperature between 300° and 500° C. The effect of such treatment consists 30 therein that hydrocarbons are formed by chemical reaction between the hydrogen and the carbon compounds of the coal, which are either liquid at ordinary temperature or have a low melting point. Only a very small portion of the carbon is volatilized in form 35 of methane at the working temperature which is materially below the proper coal distillation temperature so that in the process of this invention practically no coal distillation products are formed. Notwithstanding this, the amount of liquid products 40 formed by the process is many times greater than that obtained by the usual coal distillation and reaches nearly 100% of the carbonaceous substance of the coal, whereas the liquid products of usual coal distillation 45 generally do not exceed say 3%.

The nitrogen contained in the coal is transformed during the hydrogenation process into ammonia and ammonium compounds and the same can be recovered in 50 this form almost quantitatively.

Some of the organic compounds produced by the hydrogenation process contain oxygen and are of the phenolic type. The chief part is recovered as hydrocarbons of different boiling points, similar to petroleum distillates. 55

The unliquefied residue is a dark colored substance containing the ash of the original charge and a small proportion of carbonaceous material. 60

The period of reaction can be shortened and the output increased if a hydrocarbon capable of dissolving or diluting the resulting products, such for example as a heavy 65 commercial grade of benzene, is added to the dry material to be treated.

The process is applicable not only to natural coal and other products of natural carbonization of wood and of other vegetable material, but also to wood, peat and other vegetable material, these substances undergoing carbonization during the heating process according to this invention. Furthermore, the process is applicable also 75 to the products of coal distillation such as tar and pitch, producing therefrom compounds of lower melting-point.

In order to carry through the process an apparatus may be used which allows the 80 treatment of coal under high pressure at an elevated temperature with hydrogen or hydrogen-containing gases or hydrogen-generating substances, that is to say, substances which are capable of liberating 85 hydrogen under the operating conditions, as for example the hydrogen compound calcium, CaH.

A suitable apparatus is diagrammatically 90 shown on the annexed drawing.

1 designates a reaction vessel adapted to withstand high pressures. 2 is a charging orifice, allowing the introduction of the carbonaceous material to be treated. 3 is a vessel surrounding the reaction vessel 1 and 95 filled with molten metal 4, the melting point of which is below the required reaction temperature. 5 is a furnace for heating the metal-bath vessel 3. 6 is a high pressure 100 hydrogen container communicating with the interior of the reaction vessel 1 by a conduit 7. 8 is an exit pipe leading to a coil 9 which

opens into a vessel 10. 11 is a circulating pipe having inserted therein a pump 12. 13 is a cooler.

The operation of the device is as follows:—

- 10 The charging orifice 2 of the reaction vessel is opened and the material to be treated placed therein. This material consists either of powdered coal, or of a suspension of coal in a liquid which serves as a diluent for the products of reaction to be formed by the process. After filling the charge into the reaction vessel the orifice 2 is closed pressure-tight. Thereafter hydrogen from receptacle 6 is introduced into the reaction vessel 1 and the pressure in the reaction vessel brought to the desired degree. The furnace 5 is started and the metal bath 4 brought to the desired working temperature.
- 20 The pump 12 is put in operation so that hydrogen is circulated through the reaction vessel and the material therein. The circulation of the hydrogen effects a suitable stirring of the material under treatment.
- 25 Under the effect of heat and pressure hydrocarbons are formed within the vessel by reaction between the coal and hydrogen under high pressure, and portions of these hydrocarbons are transported with the circulating stream through the coil 9 and are condensed by the operation of the condenser 13. The condensed material accumulates within the vessel 10 from which it can be removed. The uncondensed gas consisting
- 30 nearly entirely of hydrogen is returned by the pump 12 to the reaction vessel 1. The consumed hydrogen is replaced by new gas taken from the receptacle 6. The ammonia escaping from the coal under treatment may
- 35 be retained within the receptacle 10 in any suitable manner as by any suitable absorbent.

*Examples.*

- 45 1. 400 kg. powdered coal are filled into a pressure-resisting vessel of about 400 liters capacity, which is connected to a tank in which hydrogen is held under 200 atmospheres pressure. After 15 hours the connection with the hydrogen tank is turned off and the vessel is emptied. About 10 to 15 kg. of hydrogen have then been consumed, according to the quality of coal used.

From the contents of the vessel more than 55 half of the coal can be separated from the solid residue as liquid.

The remaining part of liquid products in the solid residue can be gained by extraction.

- 60 2. 150 kg. powdered coal are placed with an equal quantity of heavy benzene in a pressure resisting vessel of about 400 liters capacity and the same is connected to a hydrogen tank. For the purpose of better

mixing, the vessel is either rotated, or the 65 contents stirred and heated to 400°.

After 12 hours the vessel is opened and the liquid produced is separated from the solid residue. Only 15% of the weight of coal employed is then left. The remaining 70 85% is dissolved in the benzene. The consumption of hydrogen is about 5 kg.

3. 400 kg. powdered coal are filled into a pressure resisting vessel of about 400 liters capacity and the same is connected to a tank 75 in which hydrogen is held under 200 atmospheres pressure and heated to about 400°. After two hours the operation is interrupted and the material removed from the vessel. It contains only a small quantity of 80 liquid substance, which is separated from the solid material. The solid material is extracted with an organic solvent such as benzene, in an extracting apparatus. After distilling the benzene, the products gained 85 by hydrogenation process and contained therein, can be extracted.

The terms "hydrogen-containing," and "hydrogen-yielding," as used in the claims, are intended to include, and do include, substances, such as liquids or gases, that impart hydrogen to the unsaturated carbon compounds in the coal, etc., as well as free hydrogen, by which the hydrogenation of the unsaturated compounds is effected, during 95 the reaction.

What we claim is:—

1. The process of treating products of carbonization of vegetable matter which consists in subjecting them to the action of hydrogen at elevated temperature of less than 100 600° centigrade and at high pressure of more than 20 atmospheres until liquid or low-melting-point reaction products of the solid carbonaceous matter are formed.

2. The process of treating products of carbonization of vegetable matter which consists in subjecting them to the action of hydrogen at a temperature from 300° to 110 500° centigrade and at high pressure of more than 20 atmospheres until liquid or low-melting-point reaction products of the solid carbonaceous matter are formed.

3. The process of treating products of carbonization of vegetable matter which consists in subjecting them to the action of hydrogen at a temperature from 300° to 115 500° centigrade and at a pressure of more than 100 atmospheres until liquid or low-melting-point reaction products of the solid 120 carbonaceous matter are formed.

4. The process of treating products of carbonization of vegetable matter which consists in reacting thereon with hydrogen at elevated temperature and high pressure until most of the solid carbonaceous substance is transformed into liquid or low-melting-point compounds.

5. The process of treating products of carbonization of vegetable matter which consists in carbonizing vegetable matter in the presence of hydrogen at elevated temperature and high pressure and continuing the hydrogen treatment until most of the solid carbonaceous substance is transformed into liquid or low-melting-point compounds. 45
6. The process of treating products of carbonization of vegetable matter which consists in reacting upon a mixture or emulsion of the carbonized material in a suspending and diluting medium with hydrogen at elevated temperature and high pressure, said suspended and diluting medium forming a liquid under working conditions. 50
7. The process of treating products of carbonization of vegetable matter which consists in subjecting them to the action of hydrogen-containing gases at an elevated temperature of less than 600° centigrade and at a high hydrogen pressure of more than 20 atmospheres until liquid or low-melting-point reaction products of the solid carbonaceous matter are formed. 55
8. The process of treating products of carbonization of vegetable matter which consists in subjecting them to the action of hydrogen-yielding substances at an elevated temperature of less than 600° centigrade and at a high hydrogen pressure of more than 20 atmospheres until liquid or low-melting-point reaction products of the solid carbonaceous matter are formed. 60
9. The process of treating coal and similar substances produced by natural or artificial carbonization, to produce liquid compounds, which comprises reacting thereon with hydrogen under increased pressure and at an elevated temperature less than 600° C. 65
10. The process of treating coal and similar substances produced by natural or artificial carbonization, to produce liquid compounds, which comprises reacting thereon with hydrogen-containing substances under increased pressure and at an elevated temperature less than 600° C. 70
11. The process of treating coal and similar substances produced by natural or artificial carbonization to produce liquid compounds, which comprises reacting thereon with hydrogen-yielding substances under increased pressure and at an elevated temperature less than 600° C. 75
12. The process of treating coal and similar substances produced by natural or artificial carbonization to produce liquid compounds, which comprises reacting thereon with hydrogen under increased pressure and at an elevated temperature and in the presence of a solvent. 80
13. The process of treating coal and similar substances produced by natural or artificial carbonization to produce liquid compounds, which comprises reacting thereon with hydrogen under increased pressure and at a temperature of about 400° C. 85
14. The process of treating coal and similar substances produced by natural or artificial carbonization to produce liquid compounds, which comprises reacting thereon with hydrogen under increased pressure and at a temperature of about 400° C., and in the presence of a solvent. 90
- In testimony whereof, we affix our signatures in presence of two witnesses. 95
- DR. FRIEDRICH BERGIUS.  
JOHN BILLWILLER.
- Witnesses:
- S. HENDY REED,  
KARL EGGERS.